

## UNITED STATES PATENT OFFICE

2,336,154

## ACID TREATMENT OF COKING COALS

Clayton S. Wolf, New Haven, Conn., assignor, by  
mesne assignments, to American Cyanamid  
Company, New York, N. Y., a corporation of  
Maine

No Drawing. Application July 2, 1940,  
Serial No. 343,553

9 Claims. (Cl. 202—20)

The present invention relates to the treatment of coking coals and more particularly it relates to a method for altering the coking characteristics of bituminous coals by treatment with chemical reagents.

In the carbonization of bituminous coals difficulties are often encountered because of intense swelling and caking of the coal when passing through the plastic temperature range. Therefore, in coking bituminous coals it is usually necessary to determine the maximum rate of temperature rise, that is, degrees per minute rise, to which the coal can be subjected while passing through the plastic temperature range without undue swelling and caking. This maximum rate of temperature rise varies considerably with different coals. For example, the Pittsburgh seam coals are high volatile-containing, highly swelling and caking coals and can only stand a temperature rise of about  $\frac{1}{2}$ ° C. per minute through the plastic temperature range. The Beckley seam coals on the other hand, are somewhat less highly swelling coking coals and can be carbonized at a temperature rise of about 2° C. per minute through the plastic range. When coking bituminous coals are formed into briquettes and then the briquettes subjected to carbonization, additional factors must be considered because some binders have swelling properties and may have a softening or fluxing action on the coal itself, or they may lack sufficient binding strength to permit the briquettes in the lower portion of the coking ovens to bear a superimposed head load of the briquettes above. It is therefore desirable that methods of altering the coking characteristics of bituminous coals be developed which will permit a higher rate of temperature rise while passing through the plastic temperature range and also which will permit the use of a wider range of binding substances in the manufacture of briquettes.

It is well known that the tendency of a given coking bituminous coal to swell and cake when subjected to carbonization can be reduced if this

coal is subjected to some form of oxidation, for example a coal which swells badly when carbonized at a temperature rise of about  $\frac{1}{2}$ ° C. per minute through the plastic range of about 300—500° C. can after oxidation be carbonized at a greater rate of temperature rise through this critical temperature range. Various methods have been proposed in the past for effecting this oxidation such as crushing the coal and heating to some predetermined practical temperature and keeping the coal elevated to this temperature for a period of time varying from 24 to 125 hours, depending upon the particular coal being treated. From a practical standpoint such a process has the serious disadvantage that it requires a long period of time to produce the desired results. An improved oxidation process is described in the copending application of William J. Kruppa, Serial No. 343,518, filed July 2, 1940, in which very finely ground coal is subjected to pressure in the presence of an oxidizing gas in a closed vessel while at the same time being maintained at an elevated temperature. In this process many coals are sufficiently oxidized in a period of only about four hours. Another method of reducing the time requirement is described in my copending application, Serial No. 343,511, filed July 2, 1940, in which the finely ground coal is heated to a temperature of about 150° C. and then subjected to alternate vacuum and atmospheric treatments in a closed vessel. In this process the coals are sufficiently oxidized in less than two hours. While the oxidizing processes described in the copending applications above have overcome the disadvantage of the unusually long periods of time that were necessary in the prior oxidation processes, they have not entirely eliminated all the commercial disadvantages in that they do require special equipment for carrying out the processes.

In accordance with the present invention I have found that the coking characteristics of swelling and caking bituminous coals can be altered by treatment with various inorganic

acids, mixtures of inorganic acids, or mixtures of inorganic acids and oxidizing salts. My process is applicable to the treatment of coking bituminous coals generally and it may be used for treating the highly swelling and caking coals such as the Pittsburgh seam coals as well as the less highly swelling coals of the Beckley seam type. When the Pittsburgh seam coals are treated by this process the coking characteristics are altered to such an extent that they can be briquetted and subjected to carbonization operations in which the temperature rise through the plastic temperature range can be carried out at the rate of at least 2° C. per minute using coal tar or pitch as a binder. Coals of the Beckley seam type can be treated by this process to alter the coking characteristics to such an extent that they can be compressed into briquettes using coal tar or pitch as the binder and then subjected to carbonization treatments in which the temperature rise permitted in the plastic temperature range is in the order of 2 to 2½° C. per minute. It is readily seen, therefore, that any bituminous coal capable of coking can be altered by my process in a manner which will permit the coals to be briquetted and carbonized under practical conditions and which also makes possible the use of a wider choice of binders.

Briefly, my invention comprises treating finely ground bituminous coals with various inorganic acids, mixtures of inorganic acids or mixtures of inorganic acids with oxidizing salts at temperatures of from 90-250° C. for about 5 to 30 minutes. The temperature at which the treatment is carried out and the rate of temperature rise will of course vary with the particular coal being treated, the acid used, % strength of acid, and also the binder which is to be used in the subsequent briquetting operations. In any event, the process can be so regulated that it is possible to predetermine the exact conditions under which the process should be carried out to effect the necessary suppression of swelling and caking tendencies of the coals. The acid treatment of the various coking bituminous coals can be so regulated that the processing rate of the coal can be increased. For example, an untreated coal which swells badly at a processing rate of 1° C. temperature rise through the plastic stage, can, after the acid treatment be processed at a rate of 2° C. per minute. The process is easily controlled and the coking characteristics of coals such as those of the Pittsburgh seam type can be altered in varying degrees. For example, the treatment can be used to change the characteristics of such coals to something in the order of a Beckley seam coal when it is desired to use sulfite liquor as a binder in the manufacture of briquettes. If coal tar or pitch is to be used as the binder, the acid treatment should be somewhat more severe in order to compensate for the swelling and slumping which accompanies the use of such a binder.

The present invention should not be confused with prior processes of treating coals with inorganic acids to react with ash-producing constituents or for the purpose of removing sulfur and phosphorous compounds from coals. These prior acid treating processes were for the purpose of removing certain objectionable constituents from the coal, whereas the present acid treating process is for the purpose of increasing the rate of processing bituminous coals in carbonization processes without undue swelling or slumping.

Among the various reagents that have been found to be useful in carrying out my process are the inorganic acids such as sulfuric, nitric, hydrochloric, perchloric, mixtures of these acids such as aqua regia or a mixture of sulfuric and nitric acids, or sulfuric acid containing a small amount of potassium permanganate or potassium chromate. The most successful acid from the standpoint of the lowest temperature required is perchloric acid, with aqua regia being about equal. From the practical standpoint, however, sulfuric is the best for commercial use due to its being comparatively cheap. The following specific tests, carried out on different coking coals will serve to illustrate the operativeness of the present invention and also the flexibility of the invention when applied to different coking coals.

A sample of Ocean coal of the Pittsburgh seam was ground to -28 mesh and then mixed with 1.6% of a 1.85 specific gravity sulfuric acid (which had been diluted with one-half its weight of water). The mixture was then stirred and heated to a temperature of about 150° C. for five minutes. The mixture was then fluxed with 8% of an acid-treated tar binder and compressed into briquettes. These briquettes were carbonized at a temperature rise of 2½° C. per minute through the plastic temperature range. At the same time there was carbonized along with these briquettes, briquettes made from the same coal ground to the same mesh but which had not been treated by fluxing with the sulfuric acid at 150° C. The briquettes made from the acid treated coal were unswollen while the ones which had not been treated were badly swollen.

In another test a sample of -28 mesh Beckley seam coal was fluxed with 1.6% of a 1.8 specific gravity sulfuric acid (diluted with one-half its weight of water). This mixture was slowly agitated and heated to a temperature of about 130° C. for about 5 minutes after which the burners were turned off and the mixture agitated until the temperature had dropped to about 125° C. Then 8% of a treated tar binder was added and fluxed thoroughly with the coal which was then transferred to a plant roll press and briquetted. The briquettes were carbonized at a rate of 2° C. per minute through the plastic temperature range. About 25% of the briquettes were appreciably swollen while the remaining 75% were only very slightly swollen and there was no sticking together of the briquettes. This Beckley seam coal cannot normally be fluxed with a tar binder, briquetted and carbonized at a temperature rise of more than 1° C. per minute. Further tests carried out on the same coal indicated that when higher temperatures of from 200-250° C. were used, a smaller amount of acid was required to produce equivalent results.

Further tests were carried out on a sample of Ocean coal in which aqua regia, nitric acid, hydrochloric acid, perchloric acid, mixtures of sulfuric and nitric acids, and mixtures of sulfuric and hydrochloric acids were used. These tests were carried out on a laboratory scale in which a 50 gram sample of the -28 mesh coal was mixed with the acid inorganic oxidizing reagent in a suitable container and then heated to the desired temperature after which the coal was fluxed with 8% of a sulfuric acid treated tar, briquetted on a hydraulic press, and carbonized in a laboratory retort at 2½° C. per minute rise through the plastic range with a superimposed steel bar head load. The results are tabulated in the following table.

Table 1

| No. | Acid used                                                                                                     | Temperature treatment     | Binder                                                         | Description of carbonized briquette                           |
|-----|---------------------------------------------------------------------------------------------------------------|---------------------------|----------------------------------------------------------------|---------------------------------------------------------------|
| 1.  | None.....                                                                                                     | None.....                 | None.....                                                      | Very badly swollen.                                           |
| 2.  | do.....                                                                                                       | 150° C.....               | H <sub>2</sub> SO <sub>4</sub> treated tar.<br>8% tar on coal. | No swelling.                                                  |
| 3.  | Aqua regia. 0.8% on coal.....                                                                                 | 150° C.....               | do.....                                                        | Very slightly swollen.                                        |
| 4.  | Aqua regia. 1.6% on coal.....                                                                                 | 150° C.....               | do.....                                                        | Noticeable improvement on No. 3.<br>No swelling.              |
| 5.  | 1.8 sp. g. H <sub>2</sub> SO <sub>4</sub> diluted with 50% H <sub>2</sub> O. 1.6% of 1.8 sp. g. acid on coal. | 150° C.....               | do.....                                                        | Somewhat swollen.                                             |
| 6.  | 1.4 sp. g. HNO <sub>3</sub> . 1.6% on coal.....                                                               | 150° C.....               | do.....                                                        | Slight swelling.                                              |
| 7.  | 50/50 H <sub>2</sub> SO <sub>4</sub> and HNO <sub>3</sub> . 1.6% on coal.....                                 | 150° C.....               | do.....                                                        | No swelling.                                                  |
| 8.  | 70% HClO <sub>4</sub> + 1/4 H <sub>2</sub> O. 1.6% on coal.....                                               | 150° C.....               | do.....                                                        | Do.                                                           |
| 9.  | 70% HClO <sub>4</sub> . 1.6% on coal.....                                                                     | None, cold<br>fluxed..... | None.....                                                      | Not as good as No. 8 showing decided benefit of 150° heating. |
| 10. | 70% HClO <sub>4</sub> . 1.6% on coal.....                                                                     | None, cold<br>fluxed..... | H <sub>2</sub> SO <sub>4</sub> treated tar.<br>8% tar on coal. | Not quite as good as No. 10.                                  |
| 11. | 70% HClO <sub>4</sub> . 0.8% on coal.....                                                                     | None, cold<br>fluxed..... | do.....                                                        | Not quite as good as No. 8.                                   |
| 12. | 70% HClO <sub>4</sub> . 1.6% on coal.....                                                                     | 100° C.....               | do.....                                                        |                                                               |

Similar laboratory tests were also conducted on a Beckley seam coal, the results of which are tabulated in the following table.

a period of at least five minutes to reduce the swelling and caking properties thereof and then compressing into briquettes and subjecting said

Table 2

| No. | Acid used                                 | Temperature treatment | Binder                                                         | Description of carbonized briquette |
|-----|-------------------------------------------|-----------------------|----------------------------------------------------------------|-------------------------------------|
| 1.  | None.....                                 | None.....             | H <sub>2</sub> SO <sub>4</sub> treated tar.<br>8% tar on coal. | Appreciably swollen.                |
| 2.  | 70% HClO <sub>4</sub> . 0.8% on coal..... | do.....               | do.....                                                        | Some improvement on No. 1.          |
| 3.  | 70% HClO <sub>4</sub> . 0.8% on coal..... | 100° C.....           | do.....                                                        | Some improvement on No. 2.          |
| 4.  | 70% HClO <sub>4</sub> . 1.6% on coal..... | 150° C.....           | do.....                                                        | No swelling.                        |

In the foregoing examples acid-treated coal tar was used as the binder in the production of briquettes. This binder comprises a 10% mixture of 60° Bé. sulfuric acid and coal tar. The present invention, however, is not limited to the use of such a binder. In briquetting operations the difficulties due to swelling and caking are usually more apparent with a pitch or tar binder than with certain other binders. It is therefore an advantage of the present invention that my pretreating process does permit the use of coal tar or pitch as a binder. On the other hand, when it is desirable to increase the head load bearing strength of briquettes, sulfite liquor may be used as the binder. In any event, the present invention can be used to alter the coking properties of any bituminous coal which will permit the coal to be coked at a faster rate of temperature rise through the plastic temperature range without swelling than would be possible if the coal had not been so treated. It is also an advantage of this invention that the process can be so regulated that in briquetting operations any of the ordinary binders may be successfully used.

What I claim is:

1. A method of making carbonized briquettes from coking coals which comprises treating badly swelling and caking coals with from about 1 to 2% of an acid inorganic oxidizing reagent at a temperature within the range of 90 to 250° C. for a period of at least five minutes to reduce the swelling and caking properties thereof and then compressing into briquettes and subjecting the briquettes to carbonization at a temperature rise of at least 2° C. per minute through the plastic temperature range.

2. A method of making carbonized briquettes from Pittsburgh seam coals which comprises treating said coals with from about 1 to 2% of an acid inorganic oxidizing reagent at a temperature within the range of 90 to 250° C. for a period of at least five minutes to reduce the swelling and caking properties thereof and then compressing into briquettes and subjecting the briquettes to carbonization at a temperature rise of at least 2° C. per minute through the plastic temperature range.

35 briquettes to carbonization at a temperature rise of at least 2° C. per minute through the plastic temperature range.

3. A method of making carbonized briquettes from Beckley seam coals which comprises treating said coals with from about 1 to 2% of an acid inorganic oxidizing reagent at a temperature within the range of 90 to 250° C. for a period of at least five minutes to reduce the swelling and caking properties thereof and then compressing into briquettes and subjecting said briquettes to carbonization at a temperature rise of at least 2° C. per minute through the plastic temperature range.

4. A method of making carbonized briquettes 50 from coking coals which coals cannot normally be compressed into briquettes and carbonized at a temperature rise of more than 1/2° C. per minute through the plastic stage without badly swelling and caking which comprises pulverizing said coal and subjecting the pulverizing coal to a treatment with from about 1 to 2% of an inorganic oxidizing acid at a temperature within the range of 90 to 250° C. for a period of at least five minutes to reduce the swelling and caking properties thereof so that when compressed into briquettes and subjected to carbonization the carbonization can be carried out at a temperature rise of at least 2° C. per minute through the plastic temperature range.

5. A method of making carbonized briquettes 55 from Pittsburgh seam coals which coals cannot normally be compressed into briquettes and carbonized at a temperature rise of more than 1/2° C. per minute through the plastic stage without badly swelling and caking which comprises pulverizing said coal and subjecting the pulverized coal to a treatment with from about 1 to 2% of an inorganic oxidizing acid at a temperature within the range of 90 to 250° C. for a period of at least five minutes to reduce the swelling and caking properties thereof so that when compressed into briquettes and subjected to carbonization the carbonization can be carried out at a temperature rise of at least 2° C. per minute through the plastic temperature range.

caking properties thereof so that when compressed into briquettes and subjected to carbonization the carbonization can be carried out at a temperature rise of at least 2° C. per minute through the plastic temperature range.

6. A method of making carbonized briquettes from Beckley seam coals which coals cannot normally be compressed into briquettes and carbonized at a temperature rise of more than  $\frac{1}{2}$ ° C. per minute through the plastic stage without badly swelling and caking which comprises pulverizing said coal and subjecting the pulverized coal to a treatment with from about 1 to 2% of an inorganic oxidizing acid at a temperature

within the range of 90 to 250° C. for a period of at least five minutes to reduce the swelling and caking properties thereof so that when compressed into briquettes and subjected to carbonization the carbonization can be carried out at a temperature rise of at least 2° C. per minute through the plastic temperature range.

7. A process according to claim 4 in which the inorganic acid is sulfuric acid.

8. A process according to claim 4 in which the inorganic acid is perchloric acid.

9. A process according to claim 4 in which the inorganic acid is aqua regia.

CLAYTON S. WOLF.